

## UNITED STATES PATENT OFFICE

EDMUND B. MIDDLETON, OF PARLIN, NEW JERSEY, ASSIGNOR TO E. I. DU PONT DE NEMOURS & COMPANY, OF WILMINGTON, DELAWARE, A CORPORATION OF DELAWARE

## DECOLORIZING FILM

No Drawing.

Application filed December 31, 1925. Serial No. 78,701.

This invention relates to a process of removing dye from tinted cellulosic materials and comprises treating the material first with a bleaching agent and then with a dye solvent 5 which preferably contains a decolorizing substance.

In the utilization or reclamation of scrap or waste pieces of cellulosic materials such as tinted celluloid or colored photographic 10 film base, etc., the presence of the tint or dye is generally objectionable and the partial or total removal of the color is often advisable before the materials are to be utilized.

It is the object of this invention to provide 15 a process for removing the dye from cellulosic materials in an efficient and economical manner without materially affecting the cellulosic base materials. Other objects and advantages will appear from the description.

20 The decolorization of the cellulosic material according to the present invention is carried out in several steps. In general, the dye is removed from the tinted cellulosic substance by first treating the substance with a 25 bleaching or an oxidizing agent which destroys all or most of the dye. The bleached material is then treated with a liquid which is a solvent for the bleached dye but is not a solvent for the cellulosic material. This 30 liquid preferably contains suspended in it a suitable decolorizing material such as bone char or activated charcoal. In this way, any of the dye remaining after the bleaching treatment is removed and the liquid solvent 35 is decolorized at practically the same time.

This invention will be described more specifically in connection with the decolorization of photographic film base, to which it is 40 particularly adapted, but is not limited to this application of the process. The tinted cellulosic photographic film base is usually dyed upon the under surface and generally is surfaced with gelatine. An illustration of 45 the procedure for decolorizing the film is as follows:

The film is generally subjected to a washing treatment whereby most of the gelatine surfacing material is dissolved off by means 50 of water or other washing liquid. After this

treatment, the washed film base is subjected to a bleaching operation.

As a suitable bleaching or oxidizing agent, a water solution of a hypochlorite is made up containing about one-tenth of one per cent of available chlorine which may be liberated by the addition of a suitable acid. The washed film is immersed in a bleaching bath of this solution until it is practically colorless or has been bleached to the desired extent. The bleaching solution may be acidified with any suitable acid immediately before or immediately after the immersion of the colored film. Or, if desired, the film may be allowed to soak in the hypochlorite solution before it is acidified. The bleaching treatment destroys most of the dye and in addition removes any gelatine remaining on the film base as a substratum or from incomplete washing.

70 After the film is bleached, it is removed from the bleaching solution and is immersed in ethyl alcohol containing decolorizing carbon such as bone char or activated charcoal. The bleached film base is soaked in the alcohol 75 containing the suspended carbon until it is free of all color. Thirty minutes' soaking is usually sufficient to remove all traces of dye. The film base is removed from the alcohol, allowed to drain, and is washed with water. 80 The adhering carbon is easily washed away, whereas with the unbleached film, some of the carbon would adhere firmly because of the gelatine present on the film. Fresh decolorizing carbon is added from time to time to take 85 the place of exhausted carbon. The exhausted carbon can be reactivated in any of the well known ways. Instead of ethyl alcohol, any other liquid may be used which is a solvent for the dye but which does not dissolve the film.

90 Instead of using a hypochlorite bleaching bath the dyed materials may be subjected to the action of moist gaseous chlorine from any suitable source. Other bleaching or oxidizing agents such as hydrogen peroxide may be used with good results.

95 The process of decolorization described generally takes place with sufficient rapidity at ordinary room temperatures to dispense 100

- with the necessity of heating during the operation. If desired, however, the process may be carried out at any suitable temperatures. Any other variations in details of the process 5 may be made without departing from the spirit of the invention. Strength of solutions and time of treating the cellulosic materials may be varied in accordance with the requirements of the material.
- 10 The dye solvent, used subsequent to the bleaching of film or tinted cellulosic material, serves a double function. The solvent not only extracts the remaining dye from the material, but it also dissolves many objectionable 15 colorless compounds, probably chlorinated compounds resulting from the reaction of chlorine with dyes, softeners and residual solvents. Many of these substances, if present, make the materials unsuitable for rec- 20lamation purposes. Ordinarily their removal would necessitate one or more separate steps or treatments, but according to the present invention these objectionable com- 25 pounds are removed in the solvent treatment.
- I claim:
1. The process of decolorizing dyed cel- lulosic films which comprises treating the films with a bleaching agent to bleach the dye and soaking the bleached product in a liquid 30 which is a solvent for the bleached dye but is not a solvent for the cellulosic material.
  2. The process of decolorizing dyed cel- lulosic films which comprises treating the films with a bleaching agent to bleach the dye and soaking the bleached product in a liquid 35 which is a solvent for the bleached dye but is not a solvent for the cellulosic material, the liquid having a decolorizing material sus- pended therein.
  - 40 3. The process of decolorizing dyed cel- lulosic films which comprises treating the films with a bleaching agent to bleach the dye and soaking the bleached product in a liquid which is solvent for the bleached dye but is 45 not a solvent for the cellulosic material, the liquid having decolorizing carbon suspended therein.
  4. The process of decolorizing dyed cel- lulosic films which comprises bleaching the 50 dye with chlorine and soaking the bleached product in a liquid which is a solvent for the bleached dye but is not a solvent for the cel- lulosic material.
  5. The process of decolorizing dyed cel- lulosic films which comprises bleaching the 55 dye with chlorine and soaking the bleached product in a liquid which is a solvent for the bleached dye but is not a solvent for the cel- lulosic material, the liquid having a decoloriz- 60 ing material suspended therein.
  6. The process of removing dye from photographic film base which comprises bleaching the dye and treating the bleached film with a bleached dye solvent which is a 65 non-solvent for the film.